

## 1

2,964,473

**ADDITIVE FOR MINIMIZING COLD SLUDGE FORMATION AND LUBRICATING OIL CONTAINING THE SAME**

Everett C. Hughes, Shaker Heights, and Harvey E. Alford Amherst, Ohio, assignors to The Standard Oil Company, Cleveland, Ohio, a corporation of Ohio

No Drawing. Filed Dec. 24, 1956, Ser. No. 630,052

2 Claims. (Cl. 252—18)

This invention relates to lubricating oil additives useful in the preparation of lubricating oil compositions having a lessened or substantially no tendency to form cold sludge and increased water tolerance, and, more particularly, to lubricating oil compositions comprising an alkaline detergent, an antioxidant, and an oil-soluble polyoxyalkylene compound.

When an engine is operated during cold weather and in light duty "stop-and-go" operations, it rarely is heated to operating temperature for any substantial portion of the driving time. When the temperatures in the crankcase are below operating temperatures, contaminants enter the crankcase by way of blow-by. These contaminants are not dissipated because of the low operating temperatures of the oil, and have an opportunity to react or to catalyze reactions in the oil. These reactions result in the formation of what is called cold sludge, a black mayonnaise-like substance. One of the most important problems today is how to combat cold sludge, because most cars used in city driving are subjected to this type of driving conditions during cold weather.

It has now been determined that when an oil containing an alkaline sulfonate type detergent and a thiophosphate type antioxidant has added thereto an oil-soluble polyoxyalkylene compound, the oil does not develop cold sludge or keeps it dispersed when the engine is operated at low temperatures for long periods of time, and in addition has the increased water tolerance. It is thought that this additive is effective in minimizing cold sludge development because it destroys the contaminants which enter the oil. These contaminants are thought to include organic peroxides and hydroperoxides. The peroxides are capable of catalyzing reactions that lead to the formation of high polymers, and it is believed that high polymers are major components of cold sludge. Accordingly, the effectiveness of the additive of the invention is thought to depend upon its ability to react with peroxides to destroy them, and the additive has been evaluated on the basis of a screening test determining decomposition of cumene hydroperoxide at 100° F.

The increased water tolerance is thought to be due to an interplay between the sulfonate detergent and the oil-soluble polyoxyalkylene compound. It is believed that the sulfonate group is adsorbed by the solids dispersed thereby in the oil. The oil-soluble polyoxyalkylene compound prevents water added to the oil from displacing this sulfonate group from the dispersed solids.

The preferred sulfonate detergent is composed of barium octadecyl sulfonate and barium carbonate. They are well known materials, and need no further description. The preferred antioxidant is zinc octyl dithiophosphate which has a molecular weight of about 321.4 and has the formula  $ZnC_8H_{17}PS(S)_2$ . It is the zinc salt of a phosphorus pentasulfide-octyl mercaptan reaction product.

The oil-soluble polyoxyalkylene compound is characterized by the following general formula:



## 2

in which R and R'' are selected from the group consisting of hydrogen, alkyl and acyl groups having from four to about twenty carbon atoms, R' is selected from the group consisting of hydrogen and alkyl groups having from one to about five carbon atoms, n is a variable small whole number from one to about four, preferably two or three, and may vary in this range even in a single long chain molecule, and y represents the number of repeating units in the chain, and may be a whole number from about five to several hundred, depending on the molecular weight.

For the purposes of the invention the character of R and R'', i.e., of the end groups of the chain, is not critical. Gum solvency properties of these compounds is attributed primarily to the oxyalkylene units which form the chain, and not to the end groups. However, although quite a wide variety of these compounds have gum solvency properties, only those with viscosities in the range of 50 to 5000 SSU at 100° F. have the necessary non-volatility and oil-solubility characteristics. These compounds are prepared by condensation of the corresponding oxides, or oxide mixtures, such as ethylene or 1,2-propylene oxide, or mixtures thereof, as is set forth more fully in U.S. Patents Nos. 2,425,755 to Roberts et al., issued August 19, 1947; 2,425,845 to Toussaint et al., issued August 19, 1947; 2,448,664 to Fife et al., issued September 7, 1948; and 2,457,139 to Fife et al., issued December 28, 1948. If R or R'' is alkyl, an aliphatic alcohol is incorporated in the reaction mixture, and if R or R'' is acyl, an aliphatic carboxylic acid is incorporated in the reaction mixtures.

Compounds in accordance with the above general formula are available commercially under the trade name "Ucon" from the Carbide and Carbon Chemicals Corporation. The compounds available commercially may have a hydroxyl group at one end of the chain and an alkyl ether or ester group at the other end of the chain, such as those of Patents Nos. 2,425,755, 2,448,664 and 2,457,139, for example, a butyl group in the Ucon LB and DLB series, but it will be understood that for the purpose of the instant invention compounds having two terminal hydroxyl groups at each end of the chain, such as those of Patent No. 2,425,845, or having two terminal alkyl ether or ester groups at each end of the chain are suitable as well. All three types of these compounds are intended to be covered by the generic term "polyoxyalkylene compound" as employed in the specification and claims.

It is essential that the polyoxyalkylene compound be oil-soluble, and have an SSU viscosity at 100° F. of from 50 to 5000. Compounds having a viscosity of less than 50 SSU are too volatile to serve as oil additives, while those having a viscosity of over 5000 SSU are too insoluble in lubricating oils to be suitable.

Very small amounts of the additives of the invention will give a marked improvement in lessening the formation of cold sludge. As little as 1.0% of the total additive mixture is effective, and amounts between 1.5% and 10.0% are preferred. Use of amounts in excess of 20.0% usually cannot be justified economically. Of the total additive mixture, the polyoxyalkylene compound is present in an amount within the range from two to sixteen parts by weight (p.b.w.). The barium octadecyl sulfonate is present in an amount within the range from 20 to 60 p.b.w., the barium carbonate in an amount within the range from 10 to 30 p.b.w., and the zinc octyl dithiophosphate in an amount within the range from 15 to 45 p.b.w.

The additives of the invention can be used to improve the cold sludge characteristics of any petroleum hydrocarbon oil of lubricating viscosity. The S.A.E. viscosities for lubricating oil range from No. 10 to No. 70. Oils

having S.A.E. Nos. 10 to 40 have a viscosity within the range from 90 to 255 SSU at 130° F., and those oils having S.A.E. Nos. 40 to 70 have a viscosity within the range from 80 to 150 SSU at 210° F. The acid-treated and solvent-extracted oils are equally useful in the compositions of the invention. The oils can be blended from suitable bright stocks and finished neutral oils of light and heavy viscosities. It is impossible here to give a complete description of the various methods used in the preparation of lubricating oils, but reference is made to the text by Georgi, entitled *Motor Oils and Engine*

5 The following example represents, in the opinion of the inventors, the best embodiment of their invention.

10 *Example*

A series of lubricating oil compositions were prepared using a lubricating oil blend of 72.5% solvent-extracted neutral thermal distillate, 300 SSU at 100° F., and 27.5% of a solvent-extracted base stock, 78 SSU at 210° F., as the base oil.

10 The properties of the base oil containing these additives are shown in Table I.

TABLE I

| Additive                                                                                                                                                                                                                           | A. NEW OIL               |                                                       |                  |                                              |             |                 |
|------------------------------------------------------------------------------------------------------------------------------------------------------------------------------------------------------------------------------------|--------------------------|-------------------------------------------------------|------------------|----------------------------------------------|-------------|-----------------|
|                                                                                                                                                                                                                                    | Viscosity SSU at 100° F. | API at 60° F.                                         | Specific Gravity | Percent Ash (SO <sub>4</sub> <sup>2-</sup> ) | pH          | Alkaline Number |
| 2.25% mixture of: 40 p.b.w. barium octadecyl sulfonate; 20 p.b.w. barium carbonate; 28 p.b.w. zinc octyl dithiophosphate                                                                                                           | 222.3                    | 30.5                                                  | 0.8737           | 0.97                                         | 7.24        | 1.05            |
| 2.25% mixture of: 40 p.b.w. barium octadecyl sulfonate; 20 p.b.w. barium carbonate; 28 p.b.w. zinc octyl dithiophosphate plus 0.25% monobutyl poly-1,2-oxypropylene glycol having a viscosity of 385 SSU at 100° F. (Flexol B-400) | 226.6                    | 30.6                                                  | 0.8730           | 0.90                                         | 8.0         | 1.69            |
| B. USED OIL                                                                                                                                                                                                                        |                          |                                                       |                  |                                              |             |                 |
| Vis. Inc. at 100° F. SSU                                                                                                                                                                                                           |                          | Percent Ash (SO <sub>4</sub> <sup>2-</sup> ) Increase |                  | pH                                           | Acid Number |                 |
|                                                                                                                                                                                                                                    | +40.1                    | 0.71                                                  |                  | 5.0                                          | 1.87        |                 |
| 2.25% mixture of: 40 p.b.w. barium octadecyl sulfonate; 20 p.b.w. barium carbonate; 28 p.b.w. zinc octyl dithiophosphate                                                                                                           | -22.3                    | 0.91                                                  |                  | 5.0                                          | 1.98        |                 |

Lubrication, published by Reinhold Publishing Corporation, New York (1950), chapter V, wherein the various types of lubricating oils are discussed fully. Any of the oils mentioned therein can be employed in the composition of the invention.

The composition of the invention is prepared simply by mixing the additives either singly or together with the oil, at room temperature. The additives are soluble or dispersible in the oil, and disperse therein instantaneously. No solvents are required.

The oils having the compositions listed below were tested for dispersancy and water tolerance.

45 The dispersancy test is a measure of the ability of the oil to hold carbon black dispersed. The oil to be tested is made up as a 5% solution thereof in benzene, and 100 ml. of the solution is placed in a glass stoppered graduate. Carbon black in increments of 0.2 gm. is added to the solution, which is then shaken for fifteen seconds and permitted to stand for five minutes in front 50 of a light source and the contents observed for a "break

TABLE II

| Example No. | Additive                                                                                                             | Percent   | Dispersancy Rating, g. Carbon Black | Water Tolerance Rating, ml. Water |
|-------------|----------------------------------------------------------------------------------------------------------------------|-----------|-------------------------------------|-----------------------------------|
| 1.....      | A mixture of: 40 p.b.w. barium octadecyl sulfonate; 20 p.b.w. barium carbonate; 28 p.b.w. zinc octyl dithiophosphate | 2.25      | 3.6                                 | 10                                |
| 2.....      | Monobutyl poly-1,2-oxypropylene glycol having a viscosity of 385 SSU at 100° F. (Flexol B-400)                       | 0.25      | 0                                   | 0                                 |
| 3.....      | Examples 1+2.....                                                                                                    | 2.25+0.25 | 3.6                                 | 100                               |

TABLE III

| Example No. | Additive                                                                                                             | Percent  | Dispersancy Rating, g. Carbon Black | Water Tolerance Rating, ml. Water |
|-------------|----------------------------------------------------------------------------------------------------------------------|----------|-------------------------------------|-----------------------------------|
| 4.....      | A mixture of: 30 p.b.w. barium octadecyl sulfonate; 20 p.b.w. barium carbonate; 38 p.b.w. zinc octyl dithiophosphate | 1.5      | 3.8                                 | 10                                |
| 5.....      | Monobutyl poly-1,2-oxypropylene glycol having a viscosity of 385 SSU at 100° F. (Flexol B-400)                       | 0.1      | 0                                   | 0                                 |
| 6.....      | do                                                                                                                   | 0.25     | 0                                   | 0                                 |
| 7.....      | do                                                                                                                   | 0.5      | 0                                   | 0                                 |
| 8.....      | Examples 4+5.....                                                                                                    | 1.5+0.1  | 4.2                                 | 50                                |
| 9.....      | Examples 4+6.....                                                                                                    | 1.5+0.25 | 4.4                                 | 90                                |
| 10.....     | Examples 4+7.....                                                                                                    | 1.5+0.5  | 4.8                                 | 40                                |

point." This point is seen as a thin upper layer of completely transparent liquid containing no carbon black particles. If no break point is observed, additional

The test cycle was repeated 16 times for a total test duration of 96 hours. The sludge cycle test results are shown in Table V.

TABLE V

| Additive                       | EXAMPLE 11<br>2.25% Mixture of: 40 p.b.w. Barium Octadecyl Sulfonate; 20 p.b.w. Barium Carbonate; 28 p.b.w. Zinc Octyl Dithiophosphate | EXAMPLE 12<br>2.25% Mixture of: 40 p.b.w. Barium Octadecyl Sulfonate; 20 p.b.w. Barium Carbonate; 28 p.b.w. Zinc Octyl Dithiophosphate; Plus 0.25% Mono-butyl Poly-1,2-Oxypropylene Glycol Having a Viscosity of 385 SSU at 100° F. (Flexol B-400) |
|--------------------------------|----------------------------------------------------------------------------------------------------------------------------------------|----------------------------------------------------------------------------------------------------------------------------------------------------------------------------------------------------------------------------------------------------|
| Blow-by c.f.m. av.             | 1.00                                                                                                                                   | 1.31                                                                                                                                                                                                                                               |
| Oil Consumption, g.            | 1,299                                                                                                                                  | 617                                                                                                                                                                                                                                                |
| Varnish Rating                 | 47.08                                                                                                                                  | 48.33                                                                                                                                                                                                                                              |
| Sludge Rating                  | 45.25                                                                                                                                  | 46.50                                                                                                                                                                                                                                              |
| Varnish plus Sludge            | 92.33                                                                                                                                  | 94.83                                                                                                                                                                                                                                              |
| Drain Oil:                     |                                                                                                                                        |                                                                                                                                                                                                                                                    |
| g. Pentane Insolubles          | 86.7                                                                                                                                   | 78.2                                                                                                                                                                                                                                               |
| g. Benzene Insolubles          | 61.3                                                                                                                                   | 46.0                                                                                                                                                                                                                                               |
| g. Acetone Methanol Insolubles | 58.5                                                                                                                                   | 45.4                                                                                                                                                                                                                                               |
| g. Soluble Resins              | 25.4                                                                                                                                   | 32.2                                                                                                                                                                                                                                               |
| g. Insoluble Resins            | 2.8                                                                                                                                    | 0.6                                                                                                                                                                                                                                                |
| Precipitated Sludge:           |                                                                                                                                        |                                                                                                                                                                                                                                                    |
| g. Pentane Insolubles          | 10.3                                                                                                                                   | 5.8                                                                                                                                                                                                                                                |
| g. Benzene Insolubles          | 5.1                                                                                                                                    | 4.0                                                                                                                                                                                                                                                |
| g. Acetone Methanol Insolubles | 4.1                                                                                                                                    | 3.2                                                                                                                                                                                                                                                |
| g. Soluble Resins              | 5.2                                                                                                                                    | 1.8                                                                                                                                                                                                                                                |
| g. Insoluble Resins            | 1.0                                                                                                                                    | 0.8                                                                                                                                                                                                                                                |
| Total Insolubles:              |                                                                                                                                        |                                                                                                                                                                                                                                                    |
| g. Pentane Insolubles          | 97.0                                                                                                                                   | 84.0                                                                                                                                                                                                                                               |
| g. Benzene Insolubles          | 66.4                                                                                                                                   | 50.0                                                                                                                                                                                                                                               |
| g. Acetone Methanol Insolubles | 62.4                                                                                                                                   | 48.6                                                                                                                                                                                                                                               |
| g. Soluble Resins              | 30.6                                                                                                                                   | 34.1                                                                                                                                                                                                                                               |
| g. Insoluble Resins            | 3.8                                                                                                                                    | 1.4                                                                                                                                                                                                                                                |
| g. Total Resins                | 34.4                                                                                                                                   | 35.5                                                                                                                                                                                                                                               |

increments of carbon black are added until there is a break point. The largest amount of carbon black which does not produce a break point is recorded as the result of the test. The test has been calibrated against various additive concentrations of dispersant additives in oil and is a measure of the dispersant or detergent properties of an oil.

The water tolerance test is an extension of the test previously described, and the solution of the oil is made up in the same way and has added to it an amount of carbon black equal to the dispersancy rating. Distilled water is then added in 10 ml. increments, and after each addition the flask is stoppered and shaken for fifteen seconds and allowed to stand five minutes. After this time, the suspension is similarly observed for a break point, and if none is observed an additional 10 ml. of water is added. This is continued until a break point is noted. The water tolerance test is important since an additive must not only have dispersant action in a dry oil but also in the presence of water because a crankcase in the winter often contains water as a result of condensation.

The dispersancy and water tolerance of the lubricating oil compositions were evaluated by the tests described.

The data show that the water tolerance and dispersancy of the barium octadecyl sulfonate-barium carbonate-zinc octyl dithiophosphate were greatly improved by addition of the polyoxypropylene glycol additive. The data also show that the polyoxypropylene glycol is not a dispersant by itself, but in the presence of the other additive it has excellent dispersancy properties. Thus, a true synergistic effect is noted.

The oils were compared in the sludge cycle test. This test is conducted in a six cylinder Chevrolet engine, unloaded, at the following cycles.

| Cycle Portion | Time, Hrs. | Speed, r.p.m. | Temperatures, ° F. |          |
|---------------|------------|---------------|--------------------|----------|
|               |            |               | Jacket             | Oil Sump |
| I             | 2          | 500           | 125                | 100      |
| II            | 2          | 2,500         | 95                 | 105      |
| III           | 2          | 2,500         | 200                | 245      |

## References Cited in the file of this patent

## UNITED STATES PATENTS

|              |                  |               |
|--------------|------------------|---------------|
| 2,369,632    | Cook et al.      | Feb. 13, 1945 |
| 2,451,345    | McNab            | Oct. 12, 1948 |
| 70 2,501,731 | Mertes           | Mar. 28, 1950 |
| 2,623,016    | Mertes           | Dec. 23, 1952 |
| 2,671,758    | Vinograd et al.  | Mar. 9, 1954  |
| 2,676,925    | Lindstrom et al. | Apr. 27, 1954 |
| 75 2,839,469 | Pfeifer          | June 17, 1958 |

UNITED STATES PATENT OFFICE  
CERTIFICATION OF CORRECTION

Patent No. 2,964,473

December 13, 1960

Everett C. Hughes et al.

It is hereby certified that error appears in the above numbered patent requiring correction and that the said Letters Patent should read as corrected below.

Columns 3 and 4, TABLE I, under the heading "USED OIL", first column thereof, for "+40.1" read -- -40.1 --; column 5, line 59, for "adata" read -- data --.

Signed and sealed this 4th day of July 1961.

(SEAL)

Attest:

ERNEST W. SWIDER

Attesting Officer

DAVID L. LADD

Commissioner of Patents